

## UNITED STATES PATENT OFFICE

MARK N. FREDENBURGH, OF EAST ORANGE, NEW JERSEY, ASSIGNOR TO WESTINGHOUSE LAMP COMPANY, A CORPORATION OF PENNSYLVANIA

## ELECTRON EMISSION MATERIAL

No Drawing.

Application filed July 20, 1928. Serial No. 294,326.

This invention relates to the art of electron discharge devices and more particularly relates to hot cathodes of the oxide coated type which are utilized in said devices and comprises essentially an improvement in the process of forming said cathodes.

In the preparation of oxide coated cathodes for electron discharge devices one of the methods used in applying the alkaline earth metal carbonates is that of spraying or painting the metal base of the cathode with a suspension of the carbonates in some volatile organic solvent or solvents in which is dissolved some binding material such as nitro-cellulose. When the organic solvent has evaporated the carbonates are held onto the cathode by the binding action of the nitrocellulose. Subsequently this organic binder is removed from the coating by heating the same in a vacuum during the exhaust procedure in the manufacture of an electron discharge device, whereupon a bonding action is thereafter established between the coating material and the metal base by effecting decomposition of the carbonates therein and conversion to oxides which react with the surface oxides of the metal base to bond thereon.

In the application of this general method of manufacturing oxide coated cathodes it has been customary to employ in forming the suspension of the carbonate material, organic solvents such as amyacetate, butylacetate or mixtures of these solvents with common alcohols, such as ethyl or methyl alcohol, to which have been added the desired proportion of nitrocellulose.

Whereas heretofore such methods have yielded excellent results and cathodes coated in this manner have had a long and useful electronic life, such results have been variable from lot to lot and day to day, depending a great deal upon production conditions.

When such suspension material is immediately employed when made excellent results are obtained therefrom. However, when such suspensions have been allowed to stand unused for various lengths of time from only a matter of a day to a week or more, the electronic efficiency of the cathodes prepared from the aged material decreases as the age there-

of increases. It is believed that such an effect is produced by some interaction between the solvent and the suspended carbonates or the solvent and the residual absorbed or adsorbed impurities of the carbonate, or that it may be produced by decomposition of the solvent material to form deleterious non-dissociable or non-decomposable compounds, which are deleterious to the electronic efficiency of the cathode prepared therefrom.

It is one of the objects of this invention to eliminate the factor of non-uniformity in product in the preparation of hot cathodes of the oxide coated type.

It is another object of this invention to eliminate the lowered emission from oxide coated cathodes that may be due to the aging of the organic suspension employed in the manufacture of said cathodes.

Another object of the invention is to provide a suspension of electron emitting material in an organic suspending medium having substantially all the advantages of prior suspensions and which is non-deteriorating with age to form compounds detrimental to the electronic emission of the alkaline earth metal component thereof.

Another object of this invention is to provide an organic solvent which may be utilized in the practice of this general coating method which is non-reactive with respect to the alkaline earth metal carbonates, or which if reactive therewith, will form compounds which are dissociable upon application of heat in an analogous manner to the alkaline earth metal carbonates.

Other objects and advantages will be apparent as the invention is more fully disclosed.

Heretofore in the prior practice it has been customary to employ as carbonate material the commercial C. P. grade of alkaline earth metal carbonates purchasable on the market. These materials were mechanically admixed in any desired proportion and suspended in the suspending medium (organic or inorganic) and applied in any desirable manner to the surface to be coated. In general the factor of adsorbed or adsorbed impurities were not allowed for and as a consequence such impurities were variable in amounts and in

identity, depending upon the method of production and prior history of the particular material employed.

I have determined that there is usually present in such commercial grades of alkaline earth metal carbonates appreciable amounts of adsorbed or absorbed impurities which are detrimental to the electronic operating efficiency of the hot cathode of an electron discharge device. Such impurities moreover are not substantially removed from such commercial grades of carbonate material by any washing or purifying process except by solution and reprecipitation of the carbonate under such controlled conditions of dilution of solution, temperature and mechanical agitation that are set forth in my copending applications Serial Nos. 292,037, filed July 18, 1928 and 293,801 filed July 18, 1928 entitled "Electron emission material", which applications are assigned to the same assignee as the present invention.

Although these impurities which may be generally classified as being alkali metal compounds such as the chlorides, nitrates or hydroxides, etc., depending upon the general method of production initially employed, may deleteriously affect the operating efficiency of the hot cathode, they are not wholly responsible for the observed loss of emission due to the aging of the organic suspension material comprising the coating, as I have determined that such a deteriorating effect is obtained when an especially purified carbonate material such as may be prepared by my copending applications Serial Nos. 292,037 and 293,801 above mentioned, is employed in the formation of such an organic suspension.

Although it is believed that the cause of the loss in electron efficiency from such organic suspensions of alkaline earth metal carbonates is due to some sort of chemical interaction or deterioration of the organic solvent to yield compounds which are deleterious to the subsequent electronic life of the hot cathode, it is obvious that it is extremely difficult to state just what the interaction or chemical combination might be, and I am not prepared at this time to predict or to calculate what reaction does take place.

I have determined, however, that by eliminating the occluded and adsorbed impurities heretofore inadvertently included in the alkaline earth metal carbonates by prior methods, by means of the special purification methods above identified and thereafter substituting for the usual organic solvents heretofore employed an organic solvent which is nonreactive with respect to the alkaline earth metal carbonates; or which if reactive therewith (over a period of time) would yield as reaction products compounds totally dissociable in vacuo by heat at the normal sealing temperatures of the hot cathodes; or

which if dissociable or decomposable under the influence of atmospheric conditions of moisture, temperatures, etc., would yield as decomposition products compounds readily dissociable and vaporizable in vacuo, the variable results heretofore obtained through the use of this general method of applying electron emitting surfaces is substantially eliminated and hot cathodes made from my improved material are uniform in operating efficiency from lot to lot and day to day irrespective of the age of the coating suspension or variations in atmospheric conditions of moisture, temperature, etc. The solvent employed should be also readily vaporizable in air and have a reasonable solubility towards a suitable binder material such as nitrocellulose. I have determined that the organic solvents diethyl carbonate ( $(C_2H_5)_2CO_2$ ) or diethyl oxalate ( $C_2O_4(C_2H_5)_2$ ) are examples of organic solvents fulfilling the provisions as above noted and may be employed in forming organic suspensions of alkaline earth metal carbonates for use in coating cathode surfaces and that suspensions employing these solvents either singly or admixed in any proportion are substantially stable for prolonged periods of time and show no evidence of deterioration or interaction of the solvent with the alkaline earth metal carbonates to yield compounds deleterious to the electron efficiency of the hot cathode prepared therefrom.

By utilizing the especially purified product as prepared by my copending applications in combination with the diethyl carbonate or diethyl oxalate, a coating composition is obtained which is superior in every respect to that heretofore obtained by prior processes, and cathodes prepared therefrom give a higher initial electron emission per unit area of surface, have a longer life, and a uniformity in production efficiency not heretofore observed.

As a specific embodiment of the nature of my invention I will describe the method I employ in forming a suspension of carbonates from material such as may be produced by my process described in copending application Serial No. 292,037, above identified. Such material is relatively dense and coarsely crystalline and requires a minimum of fluid dilutant to form a suitable suspension whereas the carbonate material produced as by my process described in copending application Serial No. 293,801, above identified, is relatively light and fluffy and requires a maximum of fluid dilutant to form a suitable suspension for coating purposes.

I first form a solution of nitrocellulose for use as a binder material as follows:

|                                  |             |
|----------------------------------|-------------|
| Nitrocellulose (parlodion) ----- | 8.0 gms.    |
| Diethyl carbonate (C. P.) -----  | 160.0 m. l. |
| Diethyl oxalate (C. P.) -----    | 40.0 m. l.  |

The nitrocellulose (parlodion) is placed in a glass bottle, the solvents are added and the mixture agitated until the nitrocellulose is thoroughly dissolved. With the use of 5 parlodion which is a very pure high grade commercial nitrocellulose product, the solution will perfectly clear and will not need any filtering. The bottle should be kept tightly stopped. This solution will be referred to 10 as binder solution #1.

I next prepare the carbonate coating suspension as follows:

Carbonate mixture 100 gms.  
15 Binder solution #1 50 m.l.  
Diethyl carbonate 50 m.l.

The coarsely crystalline carbonate mixture previously prepared as by my copending application Serial No. 293,037, above 20 identified, comprised of approximately 50% barium carbonate, 30% strontium carbonate and 20% calcium carbonate, is placed in a porcelain ball mill of 1 liter capacity, to 25 which are added 700 grams of flint pebbles (size  $\frac{1}{2}$  to  $\frac{3}{4}$ " diam.). The nitrocellulose binder and diethyl carbonate are added and the jar tightly sealed. The mill is then rotated for from 2 to 15 hours at a speed approximating 100 R. P. M. The milled mixture 30 is then poured into any suitable container and is ready for use.

The time interval of the milling operation is dependent upon what use is being made 35 of the resultant product. For use in spray methods of coating, a degree of subdivision must be obtained which will permit the coating composition to flow freely through the spray orifice. For painting and dipping operations such a degree of subdivision is not 40 required. Starting with the type of coarsely crystalline rather brittle material that is obtained by the process disclosed in my copending application I am enabled to regulate the degree of subdivision of the particles and 45 maintain the same uniformly from lot to lot and day to day, or vary it at will depending upon the ultimate use thereof.

While I have specifically described and 50 disclosed a method of forming a suspension of alkaline earth metal carbonates in an organic solvent containing a suitable binder therein, I do not wish to be limited thereby to the use of the specific components described therein. I may utilize as a solvent 55 for the nitrocellulose binder diethyl oxalate or diethyl carbonate alone, individually or in various proportionate admixtures. I may also employ as a fluid organic dilutant in the forming of the carbonate suspension either 60 diethyl carbonate or diethyl oxalate alone or admixed in any proportion. I may also vary the quantity of the proportionate admixtures of carbonate to organic suspension medium or utilize greater or lesser amounts of the 65 binder material at will, dependent upon the

material employed and the application desired thereof. I may also employ in addition to the above mentioned dilutants, a proportion of lower boiling anhydrous alcohols, particularly when the suspension is employed in the so-called spray method of coating cathodes.

These variations and all others that do not essentially depart from the nature of my invention are anticipated as may fall within the 70 scope of the invention as defined by the following claims.

What is claimed is:

1. As an article of manufacture, a coating composition for use in forming hot cathodes of the oxide coated type comprised of alkaline earth metal carbonates substantially free from adsorbed or absorbed chemical impurities, a proportion of nitrocellulose binder and diethyl carbonate as a solvent and 80 dilutant material.

2. As an article of manufacture, a coating composition for use in forming hot cathodes of the oxide coated class comprised of intimately admixed barium, strontium and calcium carbonates, a small proportion of nitrocellulose binder, and an organic solvent therefor comprised of one of the organic esters of diethyl carbonate and diethyl oxalate, in sufficient amount to form a suspension 95 for said carbonates.

3. As an article of manufacture, a suspension medium for alkaline earth metal carbonates for use in coating hot cathodes of the oxide coated type comprised of approximately equal amounts of diethyl carbonate and a solution of 20% diethyl oxalate and 80% diethyl carbonate in which is dissolved a small proportion of nitrocellulose binder.

4. The process of forming a suspension of alkaline earth metal carbonates in an organic solvent for use in the manufacture of hot cathodes of the oxide coated type, which comprises forming a mixture of alkaline earth metal carbonates in any desirable proportion substantially free of adsorbed and absorbed chemical impurities, admixing therewith diethyl carbonate in desirable amounts to form a suspension thereof, and adding thereto an organic binder material 100 comprised substantially of nitrocellulose which is soluble in said organic solvent in the form of a separate solution of the binder in diethyl carbonate containing a proportion 110 of diethyl oxalate.

In testimony whereof, I have hereunto subscribed my name this 19th day of July, 1928.

MARK N. FREDENBURGH.